

## UNITED STATES PATENT OFFICE

2,608,494

## TREATMENT OF TEXTILE FABRICS FOR IMPARTING ANTI-SHRINK PROPERTIES THERETO

Hugh vom Hove, Newport, England, assignor of one-half to Walkden Makin &amp; Co/Limited, Openshaw, Manchester, England

No Drawing. Application August 23, 1949, Serial No. 111,971. In Great Britain August 28, 1948

6 Claims. (Cl. 117—7)

1. This invention relates to improvements in processes for imparting anti-shrink properties to textile fabrics composed of or containing regenerated cellulose fibres and is particularly applicable for the treatment of crepe fabrics.

Processes for such purpose are known in which the fabric is impregnated with the pre-condensates of urea-formaldehyde resins and in which formaldehyde alone is employed to alter the hydrophilic properties, the treatment being carried out in the presence of a strong acid catalyst.

A further proposal has been to use acetone formaldehyde condensation products and it has also been suggested to use glyoxal alone or with other compounds such as the pre-condensates of urea-formaldehyde or of melamine formaldehyde in the presence of polyvinyl alcohol.

Furthermore, it has been suggested, when employing the pre-condensates of urea-formaldehyde, in order to prevent the formation of substances of high molecular structure, to carry out the process in two baths, the first bath containing urea, preferably with certain metals salts, at a concentration of about 20% and the second bath being a strong formaldehyde solution of from 20% to 40%.

The primary object of the present invention is to provide a novel process for imparting anti-shrink properties to textile fabrics containing regenerated cellulose which is carried out in two separate stages, whereby improved anti-shrink properties are imparted to such fabrics, the swelling capacity of such fabrics is reduced, and the fastness of such fabrics to light is increased.

The process according to the present invention uses two separate baths, the first bath containing either

(a) A weak organic acid which is nearly insoluble in water and having one or more alcohol-hydroxyl groups and ammonia, or

(b) A similar weak organic acid, together with ammonia, an organic amine base such as urea, thiourea, melamine, hydroxylamine, benzidine or para-phenylenediamines and the second bath containing formaldehyde of medium concentration and antimony lactate or antimony tartrate, when the first bath contains no organic amine base the amount of the organic acid should be between 1.5% to 2.5% by volume but when an organic amine base is present a much smaller amount can be employed, e. g. between 0.3% and 0.6% by volume.

Moreover when an organic amine base is present in the first bath the organic acid having one or more alcohol hydroxyl groups can be replaced by an organic acid derived from fats or fatty oils having small solubility in water such as oleic acid, caproic acid or lauric acid.

2. After complete impregnation in the first bath the fabric is dried (with or without dimensional control) at a temperature of between 60° C. and 120° C. After treatment in the second bath the fabric is dried within the same range of temperature under dimensional control such as on a stenter, giving an over stretch of 2% to 3% in the weft and overfed in the warp. The fabric is then baked at a temperature of about 150° C. for about 6 to 8 minutes and the process is completed by a short soaping treatment with the addition of a small amount of ammonia to remove any free formaldehyde remaining in the fabric.

The following examples in which the quantities are by weight are given as illustrative of the invention:

## Example 1

A green dyed crepe of 36 inch width containing 100% regenerated cellulose (viscose) in both warp and weft is impregnated at normal temperature in a bath in which the ratio of cloth to liquid is about 1:4 containing from 1.5% to 2.3% of pure ricinoleic acid, 0.35% to 0.6% concentrated ammonia and about 0.5% of a suitable known softener, the pH value of the bath being about 8.

After complete impregnation of the fabric it is squeezed in a pad mangle at a pressure of about 200 to 250 lbs. per square inch so that it contains about 80% of the liquid, and dried on a drum dryer at a temperature of from 60° C. to 120° C.

The dried fabric is then impregnated again at normal temperature in a second bath containing between 2.5% and 5% antimony lactate and 5% to 7% of formaldehyde, squeezed in a pad mangle until it contains about 80% of the liquid, dried on a stenter with about 2% stretch in the weft at a temperature of from 60° C. to 120° C. and, when dry, baked for about 6 to 8 minutes at a temperature of about 150° C.

After baking the fabric is washed in a bath containing about 0.5% of a neutral soap and about 0.5% concentrated ammonia, it is then well rinsed and dried.

The following table gives a comparison of the fabric before and after treatment in the dry state.

|                       | Tensile strength in grammes | Stretch percent | Shrinkage percent after— |     |     |
|-----------------------|-----------------------------|-----------------|--------------------------|-----|-----|
|                       |                             |                 | 1st wash                 | 2nd | 3rd |
| Untreated fabric..... | 194                         | 24.7            | 19.5                     | 20  | 20  |
| Treated fabric.....   | 199                         | 24.4            | 1.4                      | 1.4 | 1.4 |

Moreover the swelling capacity is reduced from 78% in the untreated fabric to 36% in the treated fabric.

*Example 2*

A black morrocain cloth of 36" width having a warp of 100% cellulose acetate and a weft of 50% cellulose acetate and 50% viscose is impregnated at normal temperature in a bath in which the ratio of cloth to liquid is about 1:4 containing 7.5% to 10% urea, 0.3% to 0.6% ricinoleic acid or beta oxynaphthic acid and about 0.2% concentrated ammonia.

After impregnation the fabric is dried, treated in a second bath and baked as described in Example 1.

The following table gives a comparison of the fabric in the dry state before and after treatment.

| Fabric           | Tensile strength in grammes | Stretch percent | Shrinkage percent after |     |     |
|------------------|-----------------------------|-----------------|-------------------------|-----|-----|
|                  |                             |                 | 1st Wash                | 2nd | 3rd |
| Untreated fabric | 176                         | 18.8            | 7                       | 8   | 8   |
| Treated fabric   | 174                         | 16.6            | 0                       | 0   | 0   |

The swelling capacity is reduced from 83% in the untreated fabric to 33% in the treated fabric.

It is found in many cases that the treatment according to the invention of a fabric composed of or containing regenerated cellulose not only imparts anti-shrink properties to the fabric but also increases fastness of the fabric to light.

I claim:

1. A process for imparting anti-shrink properties to textile fabrics containing at least a substantial amount of regenerated cellulose, consisting in treating such a fabric at normal temperature in a bath containing a weak organic acid selected from the group consisting of oleic, ricinoleic, caproic and lauric acid, ammonia and an organic amine base selected from the group consisting of urea, thiourea, melamine, hydroxylamine, benzidine and para-phenylenediamine, until completely impregnated therewith, drying the thus impregnated fabric, treating the dried impregnated fabric in a second bath containing formaldehyde having a substantially 20% to 40% concentration, and the antimony salt of an organic acid selected from the group consisting of lactic acid and tartaric acid, drying the impregnated fabric, and baking the dried impregnated fabric.
2. A process as defined in claim 1, wherein the organic acid employed in the first bath is ricinoleic acid.
3. A process as defined in claim 1, wherein the organic amine base employed in the first bath is urea.
4. A process as defined in claim 1, wherein the organic amine base employed in the first bath is melamine.
5. A process for imparting anti-shrink properties to textile fabrics composed mainly at least of regenerated cellulose, which comprises impregnating such a fabric at normal temperature in a

bath containing a weak organic acid selected from the group consisting of oleic, ricinoleic, caproic and lauric acid, ammonia and an organic amine base selected from the group consisting of urea, thiourea, melamine, hydroxylamine, benzidine and para-phenylenediamine, until completely impregnated therewith, drying the impregnated fabric at a temperature between 60° C. and 120° C., impregnating the dried fabric at normal temperature in a second bath containing formaldehyde having a substantially 20% to 40% concentration, and the antimony salt of a weak organic acid selected from the group consisting of lactic acid and tartaric acid until the fabric is completely impregnated therewith, drying the impregnated fabric while under an overstretch of 2% to 3% in the weft and an overfeed in the warp, baking the dried impregnated fabric at a temperature of about 150° C. for about 6 to 8 minutes, and finally giving the baked fabric a soaping treatment with the addition of an amount of ammonia sufficient to remove any free formaldehyde remaining in the fabric.

6. A process for imparting anti-shrink properties to textile fabrics composed mainly at least of regenerated cellulose, which comprises impregnating such a fabric at normal temperature in a bath of liquid containing from 0.3% to 0.6% of ricinoleic acid, 7.5% to 10% of urea, and about 0.2% concentrated ammonia, and in which bath the ratio of fabric to liquid is substantially 1:4, until impregnation of the fabric with the liquid bath is complete, drying the thus impregnated fabric at a temperature of substantially 60° C. to 120° C., subsequently impregnating such dried impregnated fabric at normal temperature in a second bath of liquid containing substantially between 2.5% and 5% of the antimony salt of an organic acid selected from the group consisting of lactic acid and tartaric acid, and 5% to 7% of formaldehyde having a concentration of substantially between 20% and 40%, until impregnation of the fabric with the liquid in the second bath is complete, drying the impregnated fabric from the second bath while under substantially 2% to 3% stretch in the weft at a temperature of substantially from 60° C. to 120° C., and baking the dried impregnated fabric for from 6 to 8 minutes at a temperature of substantially 150° C.

HUGH VON HOVE

REFERENCES CITED

The following references are of record in the file of this patent:

UNITED STATES PATENTS

| Number    | Name          | Date          |
|-----------|---------------|---------------|
| 2,165,265 | Hubert et al. | July 11, 1939 |
| 2,175,183 | Dreyfus       | Oct. 10, 1939 |
| 2,191,362 | Widmer et al. | Feb. 20, 1940 |
| 2,242,565 | Wolf          | May 20, 1941  |

FOREIGN PATENTS

| Number  | Country       | Date          |
|---------|---------------|---------------|
| 495,714 | Great Britain | Nov. 14, 1938 |
| 501,288 | Great Britain | Feb. 23, 1939 |